

# United States Patent

Copson et al.

[15] 3,645,726

[45] Feb. 29, 1972

[54] **RESISTANCE TO STRESS-CORROSION CRACKING IN NICKEL ALLOYS**

[72] Inventors: Harry R. Copson, Mahwah, N.J.; Sheldon W. Dean, Jr., Hamden, Conn.

[73] Assignee: The International Nickel Company, Inc., New York, N.Y.

[22] Filed: May 26, 1965

[21] Appl. No.: 459,050

[52] U.S. CL.....75/171, 75/124, 148/11.5, 148/12, 148/13, 148/31, 148/32, 148/134

[51] Int. Cl.....C22c 19/00

[58] Field of Search.....75/171, 170, 134, 122, 128, 75/124; 148/13, 134, 135, 136, 142, 143, 162, 32, 32.5, 37, 38, 31, 11.5, 12, 12.7

[56]

References Cited

UNITED STATES PATENTS

1,542,232 6/1925 Girin.....75/128

Primary Examiner—Richard O. Dean  
Attorney—Maurice L. Pinel

[57]

ABSTRACT

Nickel-chromium and nickel-chromium-iron-base alloys having an improved level of resistance to intergranular stress-corrosion cracking when in contact with aerated high-purity water at elevated temperatures. Alloys contain controlled amounts of aluminum, titanium, silicon and carbon. Grain size and alloy hardness correlated to further minimize stress-corrosion attack.

6 Claims, 2 Drawing Figures





INVENTORS  
 HAPPY POLLASON CORSON  
 SHELDON WILLIAMS DEAN JR.  
 BY M. L. PINEL  
 ATTORNEY

## RESISTANCE TO STRESS-CORROSION CRACKING IN NICKEL ALLOYS

The present invention relates to nickel-chromium and nickel-chromium-iron base alloys and, more particularly, to minimizing and/or overcoming the vexatious problem of stress-corrosion cracking of such alloys when exposed to a high-purity water environment.

In recent years, what must be considered as a unique problem has been reported in the literature as a result of laboratory tests (although the number of such reports has been relatively few) to the effect that nickel-chromium and nickel-chromium-iron alloys, such as those containing, inter alia, 75 to 80 percent nickel, 14 to 16 percent chromium and up to T percent or 8 percent iron, are prone to undergo stress-corrosion attack in pressurized water of high purity at temperatures on the order of about 600° F., e.g., 570° to 660° F. That there is a dearth of literature concerning the problem probably stems from the fact that the conditions causing stress-corrosion cracking are unique and specific and are not normally encountered in service. Too, it has been considered that for the most part nickel-chromium-iron alloys were thought to be rather immune to this type of corrosive attack. But the possibility of such attack coupled with the gravity of the problem and the expansion of commercial operation dictates that efforts be indeed expended to thwart or minimize the same. Data presented herein confirm that the problem can arise and little emphasis need to be added regarding the importance and significance of this phenomenon. Deleterious cracking of components and vessels and the like used in various systems of nuclear equipment wherein high-purity water is used, is indeed of no little moment.

Broadly speaking and as is well known to those skilled in the art, stress-corrosion cracking per se is a well known phenomenon. Over the years, a wealth of literature coping with the problem of stress-corrosion cracking of the austenitic nickel-chromium stainless steels has been accumulated, particularly with regard to chloride environments. While known recent avenues of approach for stainless steel were considered in seeking a solution to the problem herein, it was deemed that little by way of substantive merit would be expected, since what is apparently applicable to the stainless steels is not seemingly apposite to the instant situation. Stress-corrosion cracking of the stainless steels in chloride solutions is primarily transgranular in nature whereas the subject type of stress-corrosion cracking in nickel-chromium-iron alloys is intergranular. This factor is indicative that cracking is probably associated with some condition at the grain boundaries. Further, it has been found that AISI 304 stainless steel has upon exposure to high-purity water of high temperature also suffered stress-corrosion attack of the intergranular type in the sensitized condition.

Consideration was also given to the use of materials of very high purity, i.e., the use of extremely pure nickel, chromium and iron and not much else. This pursuit appeals more to theoretical curiosity since it is basically impractical from a commercial viewpoint. Not only is it expensive to use such materials but good commercial practice requires the use of various other elements to provide necessary deoxidizing and malleabilizing attributes and to provide, for example, good forging practice. Moreover, it is not unlikely that the mechanical properties of such alloys would be inferior.

The foregoing approaches serve to focus greater attention on appreciating the significance of the operating environmental conditions which could lead to the type of corrosive attack in question and also understanding the ostensible peculiarities or behavior of nickel-chromium-iron alloys upon exposure to such conditions. Perhaps it should be mentioned that high-purity water as contemplated herein contains not much above a total solids content of less than one part per million (p.p.m.) by weight and which has been distilled and/or deionized or otherwise treated such that it will manifest a specific resistance of about 500,000 ohm-cm. or higher. As is appreciated by those skilled in the art, this type of water is used in atomic power equipment including nuclear pressure vessels.

Certain environmental conditions have been established which either promote or are causative of inducing or creating a propensity for detrimental intergranular stress-corrosion cracking to occur in nickel-chromium-iron alloys. Aerated high-purity water (in combination with the surface condition of the alloys) is one such condition and temperature is another. Normally, high-purity water is devoid of oxygen and it is believed that the usual absence thereof has been responsible, to a considerable degree, for the lack of intergranular stress-corrosion cracking of nickel-chromium and nickel-chromium-iron alloys heretofore on a commercial scale. But the possibilities of oxygen contamination are indeed more than sufficient to warrant the necessity of finding alloys which afford a markedly higher degree of resistance to such attack.

As to temperature, if the temperature of the water is at about room temperature, stress-corrosion attack does not appear to be much of a problem. But, in commercial operation the temperature of the high-purity water is normally above room temperature and is commonly over 300° F., e.g., about 450° or 500° F., to about 660° F. and it is at such temperatures, particularly at the higher temperatures, where the occurrence of intergranular stress-corrosion attack is most likely.

As to the condition of the alloys susceptible to attack and while little is available covering the same in the published literature, it would appear that "crevices" (in combination with aerated, high-temperature, high-purity water) exert a most pronounced subversive influence in producing stress-corrosion cracking and other forms of corrosion. Whether the crevice by nature be a flaw, crack, sharp indentation or other such surface defect is rather inconsequential. The unfortunate fact remains that it is exceedingly difficult, if not impossible, to avoid or prevent the occurrence thereof. If the alloy is incapable of resisting stress-corrosion attack, there is also at least the likelihood of greater "crevice buildup" of corroded product. This would obviously interfere in applications requiring moving parts and which of necessity require adherence to observing small clearance tolerances. Thus, it can be reasonably stated without much reservation that the conditions leading to the occurrence of intergranular stress-corrosion cracking of nickel-chromium and nickel-chromium-iron alloys are at hand when aerated high-purity water of a temperature of above about 300° F. is brought into contact with certain alloys under stress and containing crevices and the like. It is to be understood, however, that other factors are undoubtedly involved. The present invention is addressed to the foregoing specific problem.

It has now been discovered that certain nickel-chromium and nickel-chromium-iron alloys of special and controlled composition afford marked resistance to intergranular stress-corrosion attack when such alloys are brought into intimate contact with aerated high-purity water at a temperature above about 300° F., e.g., 450°, to about 660° F., notwithstanding the fact that the surface of such alloys contains a surface defect, such as a crevice. It has been found that various elements in certain amounts, notably aluminum, titanium and silicon, promote the susceptibility to such attack. In addition, it has also been found that the grain size and hardness of the alloys tend to influence the behavior of the alloys in minimizing intergranular stress-corrosion cracking. An important attribute of the invention is that recourse to the utilization of highly pure constituents in making the alloys is unnecessary.

It is an object of the present invention to provide nickel-chromium and nickel-chromium-iron base alloys of special composition which manifest a high overall resistance to stress-corrosion cracking when such alloys are in contact with aerated high-purity water at a temperature above about 300° F. and up to at least about 660° F.

It is another object of the present invention to provide a process for accomplishing the foregoing.

Other objects and advantages will become apparent from the following description taken in conjunction with the accompanying drawing in which there is depicted a general relationship between hardness and grain size of alloys contem-

plated within the invention, curve AB of FIG. 1 depicting this relationship for alloys in the annealed condition and curve CD of FIG. 2 illustrating this relationship for alloys in the sensitized condition.

Generally speaking and in accordance with the present invention, stress-corrosion cracking of nickel-chromium and nickel-chromium-iron alloys to be brought into contact with aerated high-purity water, the temperature of the water being from above about 300° to about 660° F., e.g., 450° F. or 500° to about 660° F., can be greatly minimized by utilizing alloys of the following most advantageous composition (based on weight percent): about 14 to about 25 percent chromium, up to about 10 percent iron, e.g., 1 to 8 percent iron, aluminum in an amount up to 0.05 percent, e.g., about 0.005 to 0.05 percent aluminum, titanium in an amount up to 0.1 percent, e.g., about 0.01 to 0.1 percent titanium, silicon in an amount up to 0.25 percent, e.g., about 0.01 to 0.25 percent silicon, carbon in an amount up to 0.1 percent, e.g., 0.01 to 0.1 percent carbon, and the balance essentially nickel. The use of the expression "balance" or "balance essentially" in referring to the nickel content of the alloys, as will be understood by those skilled in the art, does not exclude the presence of other elements commonly present as incidental elements, e.g., deoxidizing and cleansing elements, and impurities normally associated therewith in small amounts which do not adversely affect the novel characteristics of the alloys. In this regard, it is preferred that elements such as phosphorus and sulfur be maintained at low levels as is consistent with commercial practice. Manganese can be present in amounts up to at least 2 percent, e.g., 0.1 to 1 percent.

In achieving optimum results and in addition to the aforementioned balanced chemistry of the alloys, it is advantageous to control the grain size and hardness of the alloys since relatively soft, fine-grained alloys tend to manifest greater resistance to stress-corrosion cracking. A desired correlation between grain size and hardness is generally reflected by the shaded area to the left of and/or below curves AB and CD of the attached drawing, i.e., the hardness and grain size of the alloys are preferably interrelated such that they represent a point lying within the aforesaid areas of the drawing.

Hardness and grain size, while dependent on the specific chemistry of the alloys, are also affected by heat treatment. High-temperature annealing treatments with or without the application of cold rolling are conducive to coarse-grained structures, particularly where the alloys are thereafter subjected to a sensitizing treatment. For example, alloys contemplated herein would often be welded to form a welded structure. As a result of the welding operation, the alloys would pass through a "sensitizing" temperature range of below about 1,500° to 800° F., e.g., 1,450° to 850° F. Thus, while the same alloy might manifest good resistance to intergranular stress-corrosion cracking when in the annealed condition, it might very well show cracking in the sensitized condition. Data presented herein establish that both conditions (annealed and sensitized) should be considered. Accordingly, it is thus beneficial in accordance with the invention that while the annealing treatment can be conducted over a temperature range of about 1,500° to 2,100° F., it should be carried out at a temperature of from 1,500° to about 1,700° F. and most advantageously from 1,550° to 1,650° F. At the low side of the temperature range the alloys should be held at temperature for about 1 to 2 hours or more whereas at the high side of the temperature range, e.g., 2,000° F., the alloys should be held at temperature for only a few minutes. A most satisfactory treatment in achieving a fine grain size is to cold roll the alloys up to 50 percent reduction in thickness, e.g., 25 to 40 percent, and thereafter anneal at 1,550° to 1,650° F. This treatment provides a grain on the order of about ASTM grain size No. 9 or smaller and is further beneficial in that higher amounts of carbon can be employed, if desired, than otherwise might be the case. Cold rolling is advantageous since it results in attaining an elongated grain structure and this type of grain is deemed more resistant to intergranular attack. The best condition is a soft, elongated and fine-grained, low-carbon alloy.

As has been indicated above herein, aluminum and/or titanium and/or silicon if used in excessive amounts lead to intergranular stress-corrosion cracking. It has been found that even amounts of about 0.07 percent aluminum, about 0.17 percent titanium and about 0.44 percent of silicon, respectively, have led to cracking. However, it is most important that these elements be present to provide good deoxidation, malleabilization and forging practices. Without these functional characteristics, commercial processing is, as a practical matter, rendered more difficult and/or more costly. This aspect lends emphasis to the basic impracticability of using highly pure materials. It might also be mentioned that it is considered that high amounts of aluminum and titanium promote high hardness and this in turn, as mentioned above, is conducive to stress-corrosion cracking.

Care should be exercised with regard to the carbon content of the alloys. Generally speaking, the limiting amounts of carbon present is influenced by grain size and heat treatment. It is deemed, however, that a basic criterion as to carbon content is in respect of the amount of carbon or carbide segregated at the grain boundaries in approximate inverse relation to the grain boundary area. Thus, where there is a fair number of carbides at a given grain boundary area of, say, "X," cracking might occur, whereas if the grain boundary area was "2X" or "3X," the susceptibility to cracking would be greatly lessened. With proper processing (cold rolling) and heat treatment to achieve a fine grain size of about ASTM 7 or smaller, up to 0.15 percent carbon can be employed. However, it is advantageous to maintain the carbon content at a level not greater than about 0.1 percent and preferably not greater than 0.03 percent to thereby minimize the occurrence of large amounts of carbon and/or carbide at a small grain boundary area.

Satisfactory results can also be achieved with alloys of the following composition: about 14 to about 30 percent chromium, up to about 50 percent iron, preferably not more than 25 percent iron, about 0.003 to about 0.05 percent aluminum, about 0.005 to about 0.15 percent titanium, about 0.01 to about 0.3 percent silicon, about 0.01 to about 0.15 percent carbon, and the balance essentially nickel, the nickel constituting at least 30 percent and preferably at least 35 percent of the alloys.

For the purpose of giving those skilled in the art a better understanding and/or appreciation of the invention, there is given herein data illustrative of the advantages embodied by the alloys having compositions within the invention.

A substantial number of alloy test specimens were prepared having compositions given in Table I (Alloys A to M being outside the invention and Alloys 1 to 7 being within the invention).

TABLE I

| Alloy No. | Chemical composition |      |      |      |        |        |        |
|-----------|----------------------|------|------|------|--------|--------|--------|
|           | Cr %                 | Fe % | C %  | Si % | Ti %   | Al %   | Mn %   |
| A.....    | 16.0                 | 6.9  | 0.01 | 0.03 | 0.05   | 0.07   | < 0.01 |
| B.....    | 16.0                 | 6.8  | 0.01 | 0.03 | 0.06   | 0.56   | < 0.01 |
| C.....    | 15.6                 | 6.7  | 0.01 | 0.03 | 0.09   | 2.9    | < 0.01 |
| D.....    | 15.3                 | 7.5  | 0.03 | 0.03 | 0.17   | 0.02   | < 0.01 |
| E.....    | 16.1                 | 6.4  | 0.05 | 0.19 | 0.26   | 0.07   | 0.15   |
| F.....    | 16.0                 | 7.2  | 0.05 | 0.10 | 0.32   | 0.02   | 0.29   |
| G.....    | 15.7                 | 7.1  | 0.02 | 0.10 | 0.35   | 0.01   | 2.0    |
| H.....    | 16.3                 | 6.8  | 0.10 | 0.03 | 0.96   | 0.02   | < 0.01 |
| I.....    | 15.1                 | 8.2  | 0.06 | 0.15 | 2.4    | 0.09   | 2.1    |
| J.....    | 16.0                 | 6.8  | 0.03 | 0.15 | 3.0    | 0.02   | 0.30   |
| K.....    | 15.7                 | 7.0  | 0.01 | 0.02 | 3.6    | 0.03   | 0.06   |
| L.....    | 16.0                 | 6.8  | 0.01 | 0.44 | < 0.01 | 0.02   | 0.03   |
| M.....    | 15.9                 | 7.2  | 0.05 | 0.03 | < 0.01 | < 0.01 | < 0.01 |
| *1.....   | 15.9                 | 6.7  | 0.02 | 0.04 | 0.05   | 0.03   | 0.04   |
| **1.....  | 15.9                 | 6.7  | 0.02 | 0.04 | 0.05   | 0.03   | 0.04   |
| 3.....    | 16.0                 | 6.8  | 0.01 | 0.25 | < 0.01 | 0.02   | 0.03   |
| 4.....    | 16.3                 | 7.2  | 0.01 | 0.02 | 0.08   | 0.02   | 0.07   |
| 5.....    | 16.0                 | 6.8  | 0.01 | 0.02 | < 0.01 | 0.01   | 0.26   |
| 6.....    | 16.0                 | 6.8  | 0.01 | 0.02 | < 0.01 | 0.01   | 0.54   |
| 7.....    | 15.7                 | 6.6  | 0.01 | 0.02 | < 0.01 | 0.01   | 2.2    |

\*Contained 0.007% boron.

\*\*Contained 0.002% boron.

These alloys were prepared using vacuum melting techniques and using materials of relatively high purity. The alloys were cast as 10-pound ingots. After removing surface defects, the alloys were heated to 2,200° F. and forged to flats (1 inch by 3.5 inches by 10 inches). After reheating to 2,150° F., the flats were hot rolled to a thickness of about 0.2 inch. Subsequent to conventional processing, including cold rolling to provide specimens about 0.12 inch thick, the alloys were subjected to heat treatment. Two different heat treatments were employed, one consisting of solution treating at about 1,950° F. for one-quarter hour followed by a water quench. A high-solution treatment temperature was deliberately employed to add to the severity of the test. The second treatment consisted of a sensitizing treatment whereby the specimen was heated to a temperature of about 1,300° F., held at this temperature for about one hour and then air cooled. Thus, two specimens (strips) of each alloy composition were prepared, one being subjected to the solution anneal treatment, the other being subjected to the sensitizing treatment. It was deemed necessary to test the alloys using the sensitizing heat treatment since, as referred to above herein, the alloys would be often used in this condition.

Standard autoclave testing techniques were employed and duplicate U-bend test specimens of each alloy were used. These specimens were formed by bending two flat strips simultaneously around a mandrel and inserting a bolt through the parallel legs thereof. The flat strips were about three-eighths inch in width, 0.12-inch thick and about 3.25 inches long. Prior to bending about the mandrel, an area about 0.005 inch deep and about 1 inch long was ground in the center portion of one strip. On bending about the mandrel, a tapered crevice was formed.

The test solution was aerated high-purity water (air saturated at one atmosphere) with the pH thereof having been adjusted to about pH 10.0. This test solution was placed in the autoclave and a head space having additional air was maintained. The test specimens were immersed in the solution and the autoclave sealed and brought to a test temperature of about 600° to 660° F. The autoclaves were opened about every 2 weeks and the specimens inspected for cracks, whereafter the tests were restarted with fresh solution in those instances where cracking was not visually observed. The tests were conducted generally over a period of 8 weeks and both visual and metallographic examinations of the specimens were made. The results are reported in Table II wherein the numerals indicate the time of cracking; for example, the numerals 2 and 4 indicate the specimens cracked within the first and second 2-week periods, respectively. It should be men-

tioned that if a specimen did not exhibit visual cracking, the metallographic examination was not then made; however, any specimen which did not manifest visual cracking during the full 8-week period was thereafter examined metallographically.

As illustrated by the data, a fine grain size is insufficient. Thus, Alloys H, I and K all had a grain size of ASTM No. 8 or finer and cracking occurred. In each of these three alloys, the titanium content was too high and cracking occurred regardless of the hardness, grain size relationship. Low hardness values did not necessarily result in affording resistance to intergranular stress-corrosion cracking. This is reflected, for example, by Alloys B, C and F which contained excessive amounts of aluminum (Alloys B and C) and titanium (Alloy F), wherein the annealed hardness level did not exceed 148 VHN. Alloys A, D and L additionally illustrate that aluminum, titanium and silicon in amounts as low as 0.07 percent, 0.17 percent and 0.44 percent, respectively, notwithstanding that the relationship between hardness and grain size might be represented by a point within shaded areas of curves AB and/or CD of the drawing, are conducive to cracking. Alloys E, G and J followed a rather similar pattern. Alloy M indicates that when the hardness, grain size relationship defined by curves AB and/or CD is not satisfied, cracking can ensue although the chemistry of the alloy might be within the compositional ranges described herein. However, Alloy M responded relatively well and with a lower carbon content (Alloys 1 to 7) it is considered that greater resistance to stress-corrosion cracking would be conferred. A review of all the data concerning Alloys A through M reflects that when the alloys are in the sensitized condition, there is a greater susceptibility to premature cracking. This is, of course, also indicated by the curves AB and CD.

In contrast to Alloys A through M, Alloys Nos. 1 through 7 performed satisfactorily under the same test conditions. In each case, the composition of Alloys Nos. 1 through 7 is within the scope contemplated herein as is also the preferred relationship between hardness and grain size.

It is to be observed that the present invention provides nickel-chromium and nickel-chromium-iron alloys highly resistant to intergranular stress-corrosion cracking when in contact with pressurized, aerated water at a temperature of above about 300° to about 660° F., notwithstanding that the surface of the alloys be characterized by a crevice or some such similar surface defect. The invention is also applicable in minimizing intergranular stress-corrosion cracking in aerated high-purity water at surface areas which do not contain obvious crevices. Pressure vessels, heat exchangers, steam genera-

Table II

| Alloy  | VHN** | Annealed   |               |                | Sensitized |               |                |
|--------|-------|------------|---------------|----------------|------------|---------------|----------------|
|        |       | Grain size | Cracking time |                | Grain size | Cracking time |                |
|        |       |            | Visual        | Metallographic |            | Visual        | Metallographic |
| A..... | 143   | 4          | OK, OK        | OK, OK         | 137        | 3.5           | OK, OK         |
| B..... | 141   | 6.5        | 8, OK         | C*, OK         | 145        | 6             | OK, OK         |
| C..... | 148   | 5          | 4, OK         | C, OK          | 200        | 4             | 2, OK          |
| D..... | 142   | 5.5        | OK, OK        | C*, OK         | 147        | 5             | OK, OK         |
| E..... | 151   | 5.5        | OK, OK        | OK, OK         | 148        | 4             | 2, 4           |
| F..... | 139   | 4.5        | 8, OK         | C, OK          | 141        | 4.5           | 4, OK          |
| G..... | 154   | 4          | OK, OK        | OK, OK         | 148        | 5.5           | 4, OK          |
| H..... | 223   | 9.5        | OK, OK        | OK, OK         | 207        | 9.5           | 8, OK          |
| I..... | 225   | 9          | OK, OK        | C, OK          | 260        | 9             | 4, OK          |
| J..... | 176   | 7          | OK, OK        | C, OK          | 271        | 6.5           | 4, OK          |
| K..... | 236   | 9          | OK, OK        | OK, OK         | 313        | 8             | 6, OK          |
| L..... | 149   | 5          | OK, OK        | C, OK          | 140        | 5             | OK, OK         |
| M..... | 155   | 5          | OK, OK        | OK, OK         | 154        | 6             | 8, OK          |
| 1..... | 156   | 6.5        | OK, OK        | OK, OK         | 138        | 5.5           | OK, OK         |
| 2..... | 136   | 5          | OK, OK        | OK, OK         | 136        | 5             | OK, OK         |
| 3..... | 132   | 3.5        | OK, OK        | OK, OK         | 132        | 2.5           | OK, OK         |
| 4..... | 144   | 5          | OK, OK        | OK, OK         | 141        | 5             | OK, OK         |
| 5..... | 135   | 5          | OK, OK        | OK, OK         | 130        | 5             | OK, OK         |
| 6..... | 158   | 6          | OK, OK        | OK, OK         | 143        | 6.5           | OK, OK         |
| 7..... | 139   | 4          | OK, OK        | OK, OK         | 133        | 5             | OK, OK         |

\*\* = Average hardness value.

OK = No attack in eight week test.

C = Cracks extended more than  $\frac{1}{8}$  through specimen.

C\* = Shallow cracks usually about 1 to 2 grains deep.

tion surfaces, tubing, etc., are illustrative of the type of articles which can be fabricated from the alloys of the invention. However, the present invention should not be confused with nickel-chromium and nickel-chromium-iron alloys of the age-hardening type and which contain substantial amounts of precipitation hardening ingredients such as aluminum and titanium. The alloys of the present invention are, as a practical matter, of the nonage hardening type.

As used herein and as is, of course, well known to those skilled in the art, the term "annealed condition" means the condition of the alloy upon cooling from the solution annealed condition (often referred to as simply "the annealed condition"). Similarly, sensitized condition refers to the condition of the alloy after cooling from a sensitizing treatment. It should also be mentioned that the shaded areas defined by curves AB and CD can also be expressed as the area to the left of and/or below the curves AB and CD.

Although the present invention has been described in conjunction with preferred embodiments, it is to be understood that modifications and variations may be resorted to without departing from the spirit and scope of the invention, as those skilled in the art will readily understand. Such modifications and variations are considered to be within the purview and scope of the invention and appended claims.

We claim:

1. A nickel-chromium base alloy characterized by an improved level of resistance to intergranular stress-corrosion cracking when subjected to contact with aerated high-purity water at a temperature of about 300° to about 660° F., said alloy consisting of about 14 to 25 percent chromium, up to 10 percent iron, aluminum present in an amount up to 0.05 percent, titanium present in an amount up to 0.1 percent, silicon present in an amount up to 0.3 percent, carbon in an amount up to 0.1 percent and the balance essentially nickel.

2. An alloy as set forth in claim 1 in which the aluminum is present in an amount of 0.005 to 0.05 percent, the titanium is present in an amount of 0.01 to 0.1 percent, the silicon is present in an amount of 0.01 to 0.25 percent and the carbon is

present in an amount of 0.01 to 0.03 percent, the hardness and grain size of the alloy being correlated such that when the alloy is in the annealed condition it is represented by a point falling within the shaded area defined by the curve AB of the accompanying drawing and when the alloy is in the sensitized condition it is represented by a point falling within the shaded area defined by curve CD.

3. A process for providing a nickel-chromium base alloy characterized by good resistance to intergranular stress-corrosion attack when in contact with aerated high-purity water at a temperature of about 300° to about 660° F. which comprises establishing a molten bath containing chromium, iron, aluminum, titanium, silicon, carbon and the balance essentially nickel, controlling the amounts of the respective constituents within the following ranges: about 14 to 25 percent chromium, up to 10 percent iron, aluminum present in an amount up to 0.05 percent, titanium present in an amount up to 0.1 percent, silicon present in an amount up to 0.25 percent, carbon in an amount up to 0.03 percent, and the balance essentially nickel, until the molten bath has solidified; forging the alloy and thereafter cold rolling the alloy to effect a reduction of up to about 50 percent in thickness and thereafter solution annealing said alloy at a temperature of about 1,500° to 1,700° F.

4. The process set forth in claim 3 wherein the composition, cold rolling and solution treatment are controlled such that the relationship between the hardness and grain size of the alloy is represented by a point falling within the shaded area defined by the curve AB of the accompanying drawing.

5. A process for minimizing intergranular stress-corrosion cracking of metal articles in contact with aerated high-purity water at a temperature of about 300° to about 660° F. which comprises flowing high-purity water past and in contact with such a metal article, the article being formed from an alloy in accordance with claim 1.

6. A process as set forth in claim 5 in which the article is formed from an alloy in accordance with claim 2.